

May 22, 1945.

J. S. MILLER ET AL  
BITUMINOUS COMPOSITION

2,376,798

Filed Jan. 19, 1944



FIG. 1



FIG. 2



FIG. 3

JOHN STROTHER MILLER  
JOHN L. PRESENT

INVENTORS

BY *Cleveland B. Hollingshead*  
ATTORNEY

## UNITED STATES PATENT OFFICE

2,376,798

## BITUMINOUS COMPOSITIONS

John Strother Miller, Rahway, N. J., and John L. Present, Wilmington, Del., assignors to Hercules Powder Company, Wilmington, Del., a corporation of Delaware

Application January 19, 1944, Serial No. 518,834

7 Claims. (Cl. 106—232)

This invention relates to bituminous compositions and more particularly to improved asphaltite compositions.

The asphaltites have been heretofore modified by compounding with various combinations of residual oils, vegetable oils, lubricating oils, waxes, resins, and the like to render them suitable for use in molded articles, such as battery cases, tile, insulating material, etc., in saturating and impregnating operations, and in paints and japans. The modifying agents, designed primarily to lower the softening point of the asphaltites, have not been entirely satisfactory. For example, with lowering of the softening point, the usual modifiers also produce a serious decrease in hardness or in toughness. This decrease in hardness or toughness is often accompanied by a decrease in cohesion and weathering qualities and by an increase in staining tendency.

In accordance with this invention, it has been found that compositions can be produced from the asphaltites in a manner which permits variation of the softening point while maintaining a constant degree of hardness. In other words, the invention makes possible the production of compositions having different softening points for any given hardness. Such compositions are obtained by compounding the asphaltites with a liquid ester of a rosin acid and a pine wood resin having a substantial content of gasoline-insoluble matter.

More specifically, the invention involves blending the asphaltite, pine wood resin, and liquid rosin ester in proportions such that the liquid rosin ester is in a quantity between about 10 per cent and about 50 per cent of the sum of the three said components, and the pine wood resin is in a quantity between about 10 per cent and about 35 per cent of the sum of the asphaltite and the said resin.

Having indicated the nature of the invention, the following table is given to illustrate the compositions which may be prepared. The numerical values shown are in parts by weight.

Table

|                                                      | 1  | 2  | 3  | 4  | 5  | 6  | 7  | 8  | 9  |
|------------------------------------------------------|----|----|----|----|----|----|----|----|----|
| Gilsonite (grade E)                                  | 90 | 90 | 80 | 70 | 75 | 65 | 80 | 70 | 70 |
| Pine wood resin—50% gasoline-insoluble (Belro resin) | 10 | 10 | 20 | 30 | 25 | 35 | 20 | 30 | 30 |
| Methyl abietate                                      | 70 | 25 | 70 | 70 | —  | —  | —  | —  | —  |
| Hydrogenated methyl abietate                         | —  | —  | —  | —  | 30 | 50 | —  | —  | —  |
| Triethylene glycol abietate                          | —  | —  | —  | —  | —  | —  | 20 | 35 | 10 |
| Ethyl abietate                                       | —  | —  | —  | —  | —  | —  | —  | —  | —  |

The ingredients of the different compositions shown in the table are blended by heating and stirring until homogeneous.

Examples 1, 3, and 4 are illustrative of variation in the ratio of gilsonite to pine wood resin. However, the three compositions have almost identical penetration values (hardness) while differing in softening points. The softening points are 162, 152, and 142, respectively, for the three examples and the corresponding penetration values are 19, 20, and 22. Examples 2, 7, and 9 are illustrative of compositions having greater hardness and higher softening points than those of Examples 1, 3, and 4. The remaining examples are illustrative of compositions having intermediate hardness and softening points.

The compositions of Examples 1, 3, and 4 are suitable for saturating paper. For example, 30-pound kraft paper was passed through a molten bath of the composition shown in Example 3 at 400° F. and excess asphaltite removed by doctor rolls. Rapid impregnation of the paper occurred. The same composition, heated to 350° F., was coated on 30-pound kraft paper by means of a roller coater to produce a film weighing 25–35 lbs./3000 sq. ft. The lower temperature and shorter time of contact insured a coating rather than complete impregnation of paper. A laminated article was prepared from the coated sheet by passing it with an uncoated sheet through heated rollers to secure the desired adhesion.

The compositions of Examples 2, 7, and 9 have a greater hardness at normal temperatures of use and are suitable for the preparation of molded articles. Compositions represented by Examples 5, 6, and 8 are satisfactory for saturating roofing material such as shingles and are also suitable for the production of laminated articles because of their good adhesive qualities.

The accompanying drawing serves to illustrate the effect of variation in composition upon the softening points and/or hardness.

Fig. 1 shows the effect of varying quantities of methyl abietate on the penetration values at 77° F. of different blends of gilsonite and "Belro" resin. Only one curve is shown because the effect is the same for all blends containing from 10 to 35 per cent "Belro" resin and 90 to 65 per cent gilsonite. The penetration values, which are a measure of hardness, were determined according to the standard ASTM method, D5–25 (100 g. weight for 5 seconds at 77° F.). The values shown are the depths of penetration expressed in millidecimeters, i. e., hundredths of a centimeter.

Fig. 2 shows the effect of methyl abietate on the softening points of three different blends of

gilsonite and "Belro" resin. The blends represented by the curves are as follows:

Curve A—90 parts gilsonite and 10 parts "Belro" resin

Curve B—80 parts gilsonite and 20 parts "Belro" resin

Curve C—70 parts gilsonite and 30 parts "Belro" resin.

Softening points were determined by the ring and ball method.

In Fig. 3, softening points have been plotted against penetration values at 77° F. The three curves shown represent the same blends of gilsonite and "Belro" resin as the corresponding curves in Fig. 2 with varying amounts of methyl abietate. From the softening point or penetration value at any point on either of the three curves, one may obtain the composition of the ternary mixture by referring to the corresponding curve of Fig. 2 or the single curve of Fig. 1. For example, if a point on curve C of Fig. 3 is chosen which represents a penetration value of 20, one may obtain the composition at that point by referring to Fig. 1 where it is seen that about 41 per cent by weight of methyl abietate is necessary to produce that penetration value. In a like manner, the softening point at the same point on the curve of Figure 3 can be compared with curve C of Figure 2 and the same percentage value for methyl abietate will be obtained.

From the curves of Figure 3, it can be seen that, for any given penetration value, different softening points can be obtained by varying the concentrations of the components of the mixture.

The ability to lower the softening point of gilsonite and other high melting asphaltites while maintaining a constant and desirable degree of hardness at ordinary temperatures of use is of importance because it makes possible efficient saturating and coating in molten application in the preparation of saturated, coated, laminated and molded articles. At the same time, the compositions are hard at temperatures of normal use.

Any of the asphaltites, viz., gilsonite, grahamite, and glance pitch, may be used in this invention. They differ from the asphalts and blown asphalts and are characterized by their hardness and high melting or softening points. In general, it is preferred to use gilsonite in the practice of this invention.

The rosin esters employed in this invention may be any of the esters of rosin acids which are liquids at, or slightly above, ordinary room temperatures, i. e., about 25° C. The esters may be prepared from lower aliphatic alcohols such as methyl alcohol, ethyl alcohol, propyl alcohol, isopropyl alcohol, butyl alcohol, sec-butyl alcohol, tert-butyl alcohol, hexyl alcohol, and like alcohols, higher aliphatic alcohols such as lauryl alcohol, stearyl alcohol, oleyl alcohol, etc. and rosin acids such as abietic acid, 1-pimamic acid, d-pimamic acid, sapinic acid, and mixtures of rosin acids such as occur in wood or gum rosin, or rosin which has been subjected to treatments such as polymerization, isomerization, the "Hyex" treatment (described in U. S. Patent 2,154,629 to Littman), hydrogenation, dehydrogenation, heat treatment, and the like. Polyalkylene glycols such as triethylene glycol, tetraethylene glycol, pentaethylene glycol, trimethylene glycol, tetramethylene glycol, etc., may also be used in preparing esters for use in this invention.

The quantity of the esters, which may be employed, lies within the range of about 10 to 50

per cent based upon the weight of the final composition. The amount used within this range is dependent upon the hardness desired. Quantities below 10 per cent do not have an appreciable effect on the softening point whereas quantities above 50 per cent produce undesirable degrees of softening at normal temperatures of use such as 60-90° C., i. e., penetration value at 77° F. is excessive.

As previously mentioned, the pine wood resin employed in this invention is one which contains at least 15 per cent of gasoline-insoluble material. In general, it is preferred to use a resin having at least about 35 and up to about 75 per cent gasoline-insolubles. The "Belro" resin referred to in the earlier discussion and examples is a very suitable resin obtained from the furfural solvent refining of wood rosin and contains at least 35 per cent and usually about 50 per cent of gasoline-insoluble material. Pine wood resins substantially completely insoluble in gasoline may also be used.

The quantity of resin employed is between about 10 and 35 per cent by weight based upon the combined weight of the asphaltite and resin. Quantities of resin below 10 per cent do not have an appreciable effect on the softening point whereas quantities above 35 per cent tend to increase low temperature susceptibility, i. e., cause the compositions to be brittle at temperatures of 32° F. or lower.

It will be appreciated that this invention resides in the ternary mixture and the quantities of each component may be varied within the ranges set forth depending upon the hardness and/or softening point desired in the final composition. The drawings are given only as an illustration of the compositions prepared and the effects which can be produced. Other compositions with different concentrations of each component within the specified ranges can be used to obtain additional curves. Also other materials will give slightly different sets of curves. Such curves will be useful in determining the composition necessary to produce a certain hardness and softening point.

Compositions prepared in accordance with this invention have increased utility in a wide variety of applications. Lower temperatures for melting the compositions facilitate molding, coating and laminating operations. A decrease in viscosity of the molten material, which accompanies the lowering of the softening point, increases the ease of penetration when the compositions are used for impregnation. The maintenance of hardness at normal temperatures of use while lowering the softening point increases durability in use and resistance to wear as compared to the ordinary asphalts and modified asphaltites. The compositions also have greater adhesion qualities and lessened susceptibility to low temperature effects such as embrittlement. A further advantage of this invention is the decreased staining tendency of the asphaltite compositions as compared to asphalts and softened asphaltites.

The compositions of this invention may be used in preparing thermoplastic molded articles, such as battery cases, tile, insulation materials, and the like, paints, japans and laminated articles such as laminated paper. They may also be used in coating surfaces such as building roofs, paper, etc., and in impregnating paper, fiber board, wood pulp, wood felt, roofing felt, "felt base" for flooring, glass wool, woven fabrics, and other porous objects.

What we claim and desire to protect by Letters Patent is:

1. A composition comprising a mixture of an asphaltite, pine wood resin characterized by a gasoline-insoluble matter content of at least 15 per cent, and a liquid ester of a rosin acid, the said pine wood resin being present in a quantity between about 10 per cent and about 35 per cent by weight of the sum of the asphaltite and resin, and the liquid ester being present in a quantity between about 10 per cent and about 50 per cent by weight of the said mixture.

2. A composition comprising a mixture of an asphaltite, pine wood resin characterized by a gasoline-insoluble matter content of at least 35 per cent, and a liquid ester of a rosin acid, the said pine wood resin being present in a quantity between about 10 per cent and about 35 per cent by weight of the sum of the asphaltite and resin, and the liquid ester being present in a quantity between about 10 per cent and about 50 per cent by weight of the said mixture.

3. A composition comprising a mixture of gilsonite, pine wood resin characterized by a gasoline-insoluble matter content of at least 15 per cent, and a liquid ester of a rosin acid, the said pine wood resin being present in a quantity between about 10 per cent and about 35 per cent by weight of the sum of the gilsonite and resin, and the liquid ester being present in a quantity between about 10 per cent and about 50 per cent by weight of the said mixture.

4. A composition comprising a mixture of gilsonite, pine wood resin characterized by a gasoline-insoluble matter content of at least 15 per cent, and methyl abietate, the said pine wood resin being present in a quantity between about

10 per cent and about 35 per cent by weight of the sum of the gilsonite and resin, and the methyl abietate being present in a quantity between about 10 per cent and about 50 per cent by weight of the said mixture.

5. A composition comprising a mixture of gilsonite, pine wood resin characterized by a gasoline-insoluble matter content of at least 15 per cent, and hydrogenated methyl abietate, the said pine wood resin being present in a quantity between about 10 per cent and about 35 per cent by weight of the sum of the gilsonite and resin, and the hydrogenated methyl abietate being present in a quantity between about 10 per cent and about 50 per cent by weight of the said mixture.

10 6. A composition comprising a mixture of gilsonite, pine wood resin characterized by a gasoline-insoluble matter content of at least 35 per cent, and a liquid ester of a rosin acid, the said pine wood resin being present in a quantity between about 10 per cent and about 35 per cent by weight of the sum of the gilsonite and resin, and the liquid ester being present in a quantity between about 10 per cent and about 50 per cent by weight of the said mixture.

15 7. A composition comprising a mixture of gilsonite, pine wood resin characterized by a gasoline-insoluble matter content of at least 35 per cent, and methyl abietate, the said pine wood resin being present in a quantity between about 10 per cent and about 35 per cent by weight of the sum of the gilsonite and resin, and the methyl abietate being present in a quantity between about 10 per cent and about 50 per cent by weight of the said mixture.

JOHN STROTHER MILLER.  
JOHN L. PRESENT.